

# UNITED STATES PATENT OFFICE.

ARTHUR A. BACKHAUS, OF BALTIMORE, MARYLAND, ASSIGNOR TO U. S. INDUSTRIAL  
ALCOHOL CO., A CORPORATION OF WEST VIRGINIA.

## LIQUID FUEL.

1,306,244.

Specification of Letters Patent. Patented June 10, 1919.

No Drawing.

Application filed November 28, 1917. Serial No. 204,378.

To all whom it may concern:

Be it known that I, ARTHUR A. BACKHAUS, of Baltimore, in the State of Maryland, have invented a certain new and useful Improvement 5 in Liquid Fuel, (Case 4,) and do hereby declare that the following is a full, clear, and exact description thereof.

My invention relates particularly to fuels designed to be used in any desired manner, 10 but it has application especially to fuels adapted to be used as a source of power, as for example fuels for burners and motor fuels.

The object of my invention is to provide 15 a fuel containing a petroleum hydrocarbon, as well as alcohol, and an ingredient adapted to blend the same or form a solution with the hydrocarbon and alcohol.

A further object of my invention is to provide 20 a fuel of this character, which is of such a nature that only a very small quantity of the third ingredient is found necessary.

A further object is to provide a fuel of 25 this character which contains a large percentage of the petroleum hydrocarbon, notwithstanding the small percentage of the third ingredient.

A further object is to provide a fuel of 30 this character in which the third ingredient is a fatty acid and which may, for example, be an unsaturated fatty acid.

A further object is to provide a fuel of 35 this character in which the said third ingredient is the acids obtained from linseed oil or from rape oil.

Further objects of my invention will appear from the detailed description thereof contained hereinafter.

40 While my invention is capable of being carried out in different ways, for the purpose of illustration I shall describe only certain ways of carrying out the same herein.

For example, a fuel made in accordance 45 with my invention may be made as follows:

The fuel may be comprised of

25 parts by volume of gasolene,

25 parts by volume of kerosene,

25 parts by volume of ethyl alcohol, and

50 13 parts by volume of the acids obtained from linseed oil.

As another example of my invention, the fuel may be comprised of

25 parts by volume of ethyl alcohol,

25 parts by volume of gasolene, and 55  
1½ parts by volume of the acids obtained from linseed oil.

The acids may be obtained from linseed oil by saponifying the same in any desired way. The acids thus obtained will be comprised of linolic, linolenic and oleic acids. 60

As another example of my invention, the fuel may be comprised of

25 parts by volume of gasolene,

25 parts by volume of kerosene,

25 parts by volume of alcohol, and

12 parts by volume of the acid or acids obtained from rape oil.

The acid or acids from other oils may be used instead, if desired. 70

It will be understood, however, that, instead of the gasolene and kerosene in the above examples, I may use only gasolene.

While I have described my invention above in detail, I wish it to be understood 75 that many changes may be made therein without departing from the spirit thereof.

I claim:

1. A fuel comprising a petroleum distillate, an alcohol and a fatty acid adapted to 80 blend the other constituents.

2. A fuel comprising a petroleum distillate, an alcohol and an unsaturated fatty acid adapted to blend the other constituents.

3. A fuel comprising a petroleum distillate, an alcohol and linolic acid adapted to 85 blend the other constituents.

4. A fuel comprising gasolene, an alcohol and a fatty acid adapted to blend the other constituents. 90

5. A fuel comprising gasolene, an alcohol and an unsaturated fatty acid adapted to blend the other constituents.

6. A fuel comprising gasolene, an alcohol and linolic acid adapted to blend the other constituents. 95

7. A fuel comprising gasolene, kerosene, an alcohol and a fatty acid adapted to blend the other constituents.

8. A fuel comprising gasolene, kerosene, an alcohol and an unsaturated fatty acid adapted to blend the other constituents. 100

9. A fuel comprising gasolene, kerosene, an alcohol and linolic acid adapted to blend the other constituents.

10. A fuel comprising a petroleum distillate, ethyl alcohol and a fatty acid adapted to blend the other constituents. 105

11. A fuel comprising a petroleum distillate, ethyl alcohol and an unsaturated fatty acid adapted to blend the other constituents.
  12. A fuel comprising a petroleum distillate, ethyl alcohol and linolic acid adapted to blend the other constituents.
  13. A fuel comprising gasolene, ethyl alcohol and a fatty acid adapted to blend the other constituents.
  - 10 14. A fuel comprising gasolene, ethyl alcohol and an unsaturated fatty acid adapted to blend the other constituents.
  - 15 15. A fuel comprising gasolene, ethyl alcohol and linolic acid adapted to blend the other constituents.
16. A fuel comprising gasolene, kerosene, ethyl alcohol and a fatty acid adapted to blend the other constituents.
  17. A fuel comprising gasolene, kerosene, ethyl alcohol and an unsaturated fatty acid 20 adapted to blend the other constituents.
  18. A fuel comprising gasolene, kerosene, ethyl alcohol and linolic acid adapted to blend the other constituents.

In testimony that I claim the foregoing I 25 have hereunto set my hand.

ARTHUR A. BACKHAUS.

Witnesses:

ERNEST J. WINTER,

WALTER T. SCHRINBER.